

## UNITED STATES PATENT OFFICE

2,190,331

## SCROOPING PROCESS

Hugh Harold Mosher, Nutley, N. J., and Boris Uzunoff, New York, N. Y., assignors to The Richards Chemical Works, Incorporated, Jersey City, N. J., a corporation of New Jersey

No Drawing. Application June 25, 1937  
Serial No. 150,314

3 Claims. (Cl. 91—68)

Our invention relates to novel scrooping agents and to their use in the finishing of rayon and cellulosic fibers and fabrics for the purpose of imparting to the fibers and fabrics a scroop finish which is semi-permanent in character and which will survive several detergent actions without the loss of the scroop finish.

Scroop is customarily applied to textiles by exposing the same to the action of either mineral or organic acids, particularly tartaric or citric acids. The acid hardens the periphery of the textile fibers and produces that peculiar crunchy swish known as scroop. The impartation of this character to silk is easily accomplished. Rayon fibers, however, acquire scroop with considerable difficulty and the effect when once imparted is transient and disappears after ageing the merchandise for several months. Moreover acids of a pH value of lower than 4.5 produce a gradual deterioration of the rayon fibers and may reduce the tensile strength of the yarn as much as 50 percent upon prolonged ageing.

Scroop may also be applied by impregnating the fibers with higher fatty acid esters of lower monohydric alcohols. Such a finish has the advantage of being substantially neutral and showing greater permanence than the customary acid scroops. However, these reagents impart scroop only under special conditions and cannot be universally applied as many types of fabrics resist scroop impartment by this type of finish.

We have found that the alcohols of the aliphatic series containing more than ten carbon atoms and their borates, their glycol ethers and their amines when properly dispersed with a suitable emulsificant and stabilizing agent impart a very superior scroop effect to all classes of cellulosic fabrics which likewise possess a silky hand and which will withstand several washings without a very perceptible loss of the scroopy hand.

While any aliphatic fat alcohol of more than ten carbon atoms is usable for our purpose, we have found that those alcohols of melting points between fifteen and forty degrees centigrade are most satisfactory. Where the melting point is below 15° C., the scroop effect is transient and useful only under special conditions. Where the melting point exceeds 40° C., the scroop on fabrics is apparent only when the material is maintained at a higher temperature.

We have also found that the boro esters of the raw fat alcohols equal in effectiveness the scroop influence of the corresponding fat alcohol.

We have further found that all other factors remaining constant, the aliphatic fat alcohols

bearing unsaturated bonds such as oleyl alcohol are definitely superior to those having saturated bonds.

The addition of side chain groupings in the alcohol molecules were found to be of minor importance in accentuating or inhibiting the scrooping properties of the fat alcohol emulsions.

The presence of softening agents, such as raw oils and sulphonated oils and alcohols, tend to impair the scrooping influence of the fat alcohol emulsions and it is advisable therefore, to remove these softening agents from the goods before treating the latter in accordance with our invention.

The dispersing or emulsifying agents suitable for dispersing the fat alcohols or their derivatives and esters are exemplified by the following: saturated sodium, potassium or triethanolamine soaps, sludge acid sulphonates or the naphthalene sulphonic acid esters. It is to be understood that we do not restrict ourselves to these emulsifying agents, but we have found them entirely satisfactory for our purpose.

The stabilizing agents to be associated with the fat alcohols and their esters and derivatives may be selected from among the gelatins, glues, caseins, and other proteins as well as the gums, both natural and artificial, and the starches and sugars.

The scrooping agents of our invention may be applied to rayons and other cellulosic fabrics in various ways. For example, the fat alcohols may be precipitated upon the fibers from a volatile solvent solution and the latter removed by drying. Good scrooping effects are produced in this manner, though the best results are secured by submerging the material in an aqueous suspension. The following examples serve to illustrate our invention:

*Example 1*

Twenty parts of oleyl alcohol are stirred into 100 parts of a 1% solution of triethanolamine oleate containing five parts of pure gelatine, the mixture being heated with constant stirring until a homogeneous emulsion results. The dispersion should then be passed through a colloidal mill to form a permanent emulsion.

*Example 2*

Twenty parts of technical cetyl alcohol are heated to 35° C., at which temperature the melt is slowly added to 100 parts of a 1/2% sulphonated naphthalene ester containing 2% glue with constant stirring until a permanent dispersion results. A more uniform emulsion will result by

passing the dispersion through a colloidal machine.

*Example 3*

5 Lauryl alcohol is borated by heating the fat alcohol above 150° C. with 12% boric acid. The resultant lauryl borate is then dispersed with the isopropyl naphthalene sulphonic acid, and passed through a colloid mill to insure a semi-permanent dispersion. Twenty-five percent emulsions of 10 lauryl alcohol are secured through the use of as little as one-half percent of naphthalene ester.

*Example 4*

15 Technical cetyl alcohol is first borated by exposing the raw alcohol and boric acid to a temperature of between 140 and 160° C. The borated alcohol is then dispersed in a solution containing gelatin and triethanolamine soap and greater permanence secured by passage through a 20 colloid mill. The composition of such emulsion is:

|                           | Per cent |
|---------------------------|----------|
| Cetyl alcohol borate      | 25       |
| Gelatin                   | 1        |
| 25 Triethanolamine oleate | ½        |

Rayon passed through the mixture acquires a soft, silky, scroppy hand.

If it is desired to impart a silky scroop-like finish to a rayon fabric, the fabric is scoured and dyed in the conventional manner and completely freed from all oil and other softening agents.

The material is then passed through a 5% aqueous emulsion of the fat alcohol suspension prepared as in any of the foregoing examples, 35 extracted and dried.

Our invention is applicable to the treatment of not only rayon but of all types of cellulosic fabric such as rayon velvets, spun rayon fabrics, acetate rayon material and all classes of cotton goods.

Other types of finishing ingredients, as for example waxes, sizes, sugars, etc., may be applied with the fat alcohol dispersions, but use of softening agents is undesirable.

What we claim is:

1. The herein described method of applying 10 scroop to prefinished cellulose textile material, which method comprises the steps of removing all softening agents from the material, and then treating the material with an aqueous emulsion of about 1% to 1 1/4% of a compound selected from 15 the class consisting of the aliphatic alcohols having more than ten carbon atoms in the molecule and having melting points between 15° and 40° C. and the borates and amides of said alcohols, 20 while excluding softening agents.

2. A method, as claimed in claim 1, in which said emulsion also contains from about 0.02% to about 0.03% of an emulsifying agent and from about 0.05% to about 0.3% of a stabilizing agent.

3. A method, as claimed in claim 1, in which 25 said emulsion also contains from about 0.02% to about 0.03% of an emulsifying agent selected from the class consisting of saturated sodium, potassium and triethanolamine soaps, sludge acid sulphonates and naphthalene sulphonic acid esters, 30 and from about 0.05% to about 0.3% of a stabilizing agent selected from the class consisting of gelatins, glues, caseins, gums, starches and sugars.

HUGH HAROLD MOSHER. 35  
BORIS UZUNOFF.